

## UNITED STATES PATENT OFFICE

CAMILLE DREYFUS, OF NEW YORK, N. Y.

## PILE FABRIC

No Drawing.

Application filed July 16, 1930. Serial No. 468,461.

This invention relates to pile fabrics and relates more particularly to pile fabrics having a pile of yarns of organic derivatives of cellulose.

5 An object of my invention is to produce more permanent effects in pile fabrics containing yarns of cellulose acetate or other organic derivatives of cellulose. Another object of my invention is to prepare panne velvet 10 or other fabric having a crushed pile, wherein in the tendency of the pile to rise is reduced. A further object of my invention is to prepare a pile fabric of relatively cheap construction having the pile firmly held in the 15 back of the fabric. Other objects of this invention will appear from the following detailed description.

Pile fabrics as ordinarily made present 20 some disadvantages which render the same more or less undesirable for some purposes. Thus in the case of panne velvet or other fabric having a pile which is laid or flattened down as to be more or less parallel to the face of the fabric, often the pile tends to rise 25 after use so that uneven lustre effects are produced. Moreover when the pile yarn is made of cellulose acetate or other smooth surface fibres, the pile tends to slip out from the face of the fabric unless it is anchored 30 at more than one point.

I have found that more permanent effects 35 may be obtained in pile fabric containing yarns of cellulose acetate or other organic derivatives of cellulose by taking advantage of the thermoplastic or plastic nature of such yarns. Thus by employing a solvent or softening agent and/or heat and pressure in the treatment of pile fabric containing organic derivative of cellulose yarn preferably 40 in the pile, I can make panne velvet or other crushed pile fabric, wherein the pile remains relatively permanently in the flattened position, and I can also cause the pile yarn of a relatively cheap construction, wherein the 45 individual pile is anchored at only one point in the fabric, to be held fast in such fabric.

In accordance with my invention I produce 50 more permanent effects in pile fabric containing yarns of cellulose acetate or other organic derivatives of cellulose by deform-

ing at least part of the yarn by plastic or thermoplastic action and then permitting the same to set.

While this invention will be described in connection with fabric containing yarns of cellulose acetate and particularly an acetone soluble cellulose acetate, it is equally applicable to fabrics containing yarns of other organic derivatives of cellulose such as cellulose esters and cellulose ethers. Examples 55 of such cellulose esters are cellulose formate, cellulose propionate or cellulose butyrate, while examples of cellulose ethers are ethyl cellulose, methyl cellulose or benzyl cellulose. The pile yarns preferably are made of 60 cellulose acetate. The fabric may consist wholly of yarns of cellulose acetate but the back thereof may contain yarns of other fibres such as natural silk, cotton or reconstituted cellulose, while the pile may consist 65 solely of cellulose acetate yarn, or of a mixture of cellulose acetate yarn and yarn of such other fibers.

As agencies for softening the cellulose acetates yarn, softening or swelling agents 75 may be employed, the expedients of heat and pressure, or both softening or swelling agents and heat and pressure.

The fabric to be treated may be sprayed 80 with, dipped in, or otherwise impregnated with a liquid which acts as a softening or swelling agent for the cellulose acetate material. Examples of such softening or swelling agents are solutions of solvents for the cellulose acetate in diluents. Thus the 85 solvents such as acetone, diacetone alcohol, cyclohexanone, acetic acid or ethyl lactate may be diluted with non-solvents such as water or benzol in such proportions that the resulting mixture has a softening or restricted solvent action on the cellulose acetate. A specific example of such material is an aqueous solution of acetone containing from 10 90 to 50% of acetone.

For the purpose of softening a cellulose acetate yarn, non-volatile softening agents 95 such as triacetin, monomethyl xylene sulfonamid, triphenyl phosphate and the like may be dissolved in suitable solvents such as benzol or even water and the resulting solu- 100

tion employed for treating the fabric. Swelling agents, such as ethyl alcohol or methyl alcohol may also be used for this purpose. The softening or swelling agents may 5 also contain lubricants such as oleic acid, olive oil and the like.

Preferably but not necessarily after the application of the softening or swelling agent to the pile fabric, the same is treated 10 under heat and pressure, such as by means of heated calender rolls or other heated pressing devices, whereby the yarn of cellulose acetate is further softened and deformed. Upon the removal of the heat and 15 pressure, and if necessary subsequent removal of the softening or swelling agents, permanent effects are imparted to the pile fabric. In some cases heat and pressure, without the use of a softening or swelling 20 agent may be employed in this invention.

One application of this invention is in the making of panne velvet or other pile fabric wherein the pile is laid or flattened down, that is the pile yarn occupies a position 25 which is not at right angles to the plane of the face of the fabric. In this case the pile fabric is treated with the softening or swelling agent and then pressed between hot calender rolls, or the fabric may be subjected to the action of the hot calender rolls 30 without previous treatment with the softening or swelling agent. In either case, the temperature of the calender rolls will be such that the yarn of cellulose acetate will 35 be softened. Under the conditions of treatment, the softened yarns are pressed down under pressure and since they are in a plastic condition, upon removal from the calender rolls they set permanently. The pile 40 of the fabric so treated does not tend to rise on subsequent use.

In another application of this invention, instead of flattening the whole surface of the pile by smooth calender rolls, the surface 45 may be crushed only locally by means of engraved or embossed rollers or other devices having suitable designs, to form crushed velvets or plush having the appearance of broad-tail or other furs and the like. Because of the nature of treatment, the effect is substantially permanent. Such material is useful for making coats and as 50 a drapery or upholstery fabric.

Another application of this invention is 55 in fixing more permanently the pile yarn in a fabric of relatively cheap construction. Yarn of cellulose acetate is relatively smooth and therefore in order to anchor such yarn when used as a pile, it is necessary that the loops thereof be held in at least two places by the yarn of the back of the fabric. By the present invention, a pile fabric having the pile held in only one place by the yarn of the back, that is where- 60 in the pile yarn has a more or less V shape

may be treated, and by the plastic or thermoplastic action, the pile yarn is firmly held in place.

It is to be understood that the foregoing description is given merely by way of illustration, and that many variations may be made therein without departing from the spirit of my invention.

Having described my invention, what I claim and desire to secure by Letters Patent 75 is:

1. Method of anchoring pile yarn more permanently in a pile fabric comprising applying to a pile fabric containing pile yarns of organic derivatives of cellulose, a substance that has at least a softening or restricted solvent action on the organic derivative of cellulose and then permitting the organic derivative of cellulose to harden. 80

2. Method of anchoring pile yarn more permanently in a pile fabric comprising applying to a pile fabric containing pile yarns of cellulose acetate a substance that has at least a softening or restricted solvent action on the cellulose acetate and then permitting the cellulose acetate to harden. 85

3. Method of anchoring pile yarn more permanently in a pile fabric comprising applying to a pile fabric containing pile yarns of cellulose acetate an aqueous solution of acetone and then permitting the cellulose acetate to harden. 90

4. Method of improving the qualities of pile fabrics having pile yarns of organic derivatives of cellulose which comprises applying thereto a substance having a softening or restricted solvent action on the organic derivatives of cellulose, bending the pile yarns and then permitting the same to harden, whereby the pile becomes substantially permanently anchored in a deflected position. 100

5. Method of improving the qualities of pile fabrics having pile yarns of cellulose acetate which comprises applying thereto a substance having a softening or restricted solvent action on the cellulose acetate, bending the pile yarns and then permitting the same to harden, whereby the pile becomes substantially permanently anchored in a deflected position. 110

6. Method of improving the qualities of pile fabrics having pile yarns of organic derivatives of cellulose which comprises applying thereto a substance having a softening or restricted solvent action on the organic derivatives of cellulose, bending the pile yarns by applying pressure thereto and then permitting the same to harden, whereby the pile becomes substantially permanently anchored in a deflected position. 120

7. Method of improving the qualities of pile fabrics having pile yarns of cellulose acetate which comprises applying thereto a substance having a softening or restricted 130

solvent action on the cellulose acetate, bending the pile yarns by applying pressure thereto and then permitting the same to harden, whereby the pile becomes substantially permanently anchored in a deflected position.

8. Method of improving the qualities of pile fabrics having pile yarns of cellulose acetate which comprises applying thereto a substance having a softening or restricted solvent action on the cellulose acetate, bending the pile yarn by applying pressure thereto at elevated temperatures and then permitting the same to harden, whereby the pile becomes substantially permanently anchored in a deflected position.

9. Method of improving the qualities of pile fabrics having pile yarns of cellulose acetate which comprises applying thereto an aqueous solution of acetone, bending the pile yarns by applying pressure thereto at elevated temperatures and then permitting the same to harden, whereby the pile becomes substantially permanently anchored in a deflected position.

10. Pile fabric comprising pile yarns of organic derivatives of cellulose, the pile being adherent to the base fabric.

11. Pile fabric comprising pile yarns of cellulose acetate, the pile being adherent to the base fabric.

In testimony whereof, I have hereunto subscribed my name.

CAMILLE DREYFUS.

35

40

45

50

55

60

65